



US005905021A

# United States Patent [19]

Anderson et al.

[11] Patent Number: 5,905,021

[45] Date of Patent: May 18, 1999

[54] **IMAGING ELEMENT COMPRISING AN ELECTRICALLY-CONDUCTIVE LAYER CONTAINING CONDUCTIVE FINE PARTICLES AND WATER-INSOLUBLE POLYMER PARTICLES CONTAINING SULFONIC ACID GROUPS**

[75] Inventors: **Charles Chester Anderson; Yongcui Wang, both of Penfield; Mario Dennis DeLaura, Hamlin, all of N.Y.**

[73] Assignee: **Eastman Kodak Company, Rochester, N.Y.**

[21] Appl. No.: **08/598,590**

[22] Filed: **Feb. 12, 1996**

[51] **Int. Cl.<sup>6</sup> G03C 1/85**

[52] **U.S. Cl. 430/530; 430/527; 430/529; 430/536; 430/631; 430/950; 430/63; 430/215; 430/262; 430/271.1**

[58] **Field of Search 430/63, 215, 262, 430/271.1, 527, 529, 530, 536, 631, 950**

## [56] References Cited

### U.S. PATENT DOCUMENTS

3,773,517 11/1973 Dodwell 430/628

4,294,739 10/1981 Upson et al. .... 430/527  
4,510,238 4/1985 Kingston et al. .... 430/631  
5,061,595 10/1991 Gingello et al. .... 430/961  
5,175,073 12/1992 Gingello et al. .... 430/950  
5,279,933 1/1994 Gingello et al. .... 430/509  
5,340,676 8/1994 Anderson et al. .... 430/63  
5,372,921 12/1994 Gingello et al. .... 430/509  
5,447,832 9/1995 Wang et al. .... 430/523  
5,459,021 10/1995 Ito et al. .... 430/527  
5,466,567 11/1995 Anderson et al. .... 430/530  
5,529,893 6/1996 Valsecchi et al. .... 430/529

*Primary Examiner*—Geraldine Letscher  
*Attorney, Agent, or Firm*—Carl F. Ruoff; Alfred P. Lorenzo

## [57] ABSTRACT

Imaging elements, such as photographic, electrostatographic and thermal imaging elements, comprised of a support, an image-forming layer and an electrically-conductive layer consisting essentially of electrically-conductive fine particles, such as antimony-doped tin oxide particles and, as a binder, water-insoluble polymer particles containing sulfonic acid groups. The use of water-insoluble polymer particles containing sulfonic acid groups as a binder in the electrically-conductive layer provides a layer with a high degree of conductivity at low concentrations of electrically-conductive fine particles.

**21 Claims, No Drawings**

**IMAGING ELEMENT COMPRISING AN ELECTRICALLY-CONDUCTIVE LAYER CONTAINING CONDUCTIVE FINE PARTICLES AND WATER-INSOLUBLE POLYMER PARTICLES CONTAINING SULFONIC ACID GROUPS**

**CROSS-REFERENCE TO RELATED APPLICATIONS**

Copending commonly-assigned U.S. Provisional Patent Application Ser. No. 60/000236, filed Jun. 15, 1995, "Imaging Element Comprising An Electrically-Conductive Layer With Enhanced Abrasion Resistance" by Charles C. Anderson, Yongcui Wang, James L. Bello and Mario D. DeLaura describes imaging elements containing an electrically-conductive layer comprising electrically-conductive fine particles and gelatin-coated water-insoluble polymer particles.

Copending commonly-assigned U.S. patent application Ser. No. 08/599,908, filed Feb. 12, 1996, "Imaging Element Comprising An Electrically-Conductive Layer Containing Conductive Fine Particles And Water-Insoluble Polymer Particles Of Specified Shear Modulus" by Charles C. Anderson, Yongcui Wang and Mario D. DeLaura describes imaging elements containing an electrically-conductive layer consisting essentially of electrically-conductive fine particles and, as the binder, water-insoluble polymer particles that have a shear modulus that provides enhanced performance.

**FIELD OF THE INVENTION**

This invention relates in general to imaging elements, such as photographic, electrostatographic and thermal imaging elements, and in particular to imaging elements comprising a support, an image-forming layer and an electrically-conductive layer. More specifically, this invention relates to such imaging elements having an electrically-conductive layer containing electrically-conductive fine particles and, as the binder, water-insoluble polymer particles containing sulfonic acid groups that provide enhanced performance.

**BACKGROUND OF THE INVENTION**

A variety of problems associated with the formation and discharge of electrostatic charge during the manufacture and use of photographic films are well recognized in the photographic industry. These electrostatic charges are generated by the highly insulating polymeric film bases such as as polyester and cellulose acetate during winding and unwinding operations associated with the photographic film manufacturing process and during the automated transport of photographic films in film cassette loaders, cameras, and film processing equipment during use of the photographic film product.

It is well known that electrostatic charges can be effectively controlled or eliminated by incorporating one or more electrically-conductive antistatic layers in the photographic film. A wide variety of conductive materials can be incorporated into antistatic layers to provide a wide range of conductivity and antistatic performance. Typically, the antistatic layers for photographic applications employ materials which exhibit ionic conductivity where the charge is transferred by the bulk diffusion of charged species through an electrolyte. Antistatic layers comprising inorganic salts, ionic conductive polymers, and colloidal metal oxide sols

stabilized by salts have been described. U.S. Pat. No. 4,542,095 discloses antistatic compositions for use in photographic elements wherein aqueous latex compositions are used as binder materials in conjunction with polymerized alkylene oxide monomers and alkali metal salts as the antistatic agents. U.S. Pat. No. 4,916,011 describes antistatic layers comprising ionically conductive styrene sulfonate interpolymers, a latex binder, and a crosslinking agent. U.S. Pat. No. 5,045,394 describes antistatic backing layers containing Al-modified colloidal silica, latex binder polymer, and organic or inorganic salts which provide good writing or printing surfaces. The conductivities of these ionic conductive antistatic layers are very dependent on humidity and film processing. At low humidities and after conventional film processing the antistatic performance is substantially reduced or ineffective.

Antistatic layers employing electronic conductors have also been described. The conductivity of these materials depends on primarily electronic mobilities rather than ionic mobilities and the conductivity is independent of humidity. Antistatic layers which contain conjugated polymers, semi-conductive metal halide salts, conductive carbon or semi-conductive metal oxide particles have been described. It is characteristic of these electronically conductive materials to be highly colored or have high refractive index. Thus, providing highly transparent, colorless antistatic layers containing these materials poses a considerable challenge.

U.S. Pat. No. 3,245,833 describes conductive coatings containing semiconductive silver or copper iodide dispersed as 0.1  $\mu$ m or less particles in an insulating film-forming binder exhibiting surface resistivities of  $10^2$  to  $10^{11}$   $\Omega$  per square. However, these coatings must be overcoated with a water-impermeable barrier layer to prevent the loss of conductivity after film processing since these semiconductive salts are solubilized by conventional film processing solutions.

Conductive layers comprising inherently conductive polymers such as polyacetylene, polyaniline, polythiophene, and polypyrrole are described in U.S. Pat. Nos. 4,237,194, JP A2282245, and JP A2282248, but, these layers are highly colored.

Conductive fine particles of crystalline metal oxides dispersed with a polymeric binder have been used to prepare humidity insensitive, conductive layers for various imaging applications. Many different metal oxides are alleged to be useful as antistatic agents in photographic elements or as conductive agents in electrographic elements in such patents as U.S. Pat. Nos. 4,275,103, 4,394,441, 4,416,963, 4,418,141, 4,431,764, 4,495,276, 4,571,361, 4,999,276, 5,368,995 and 5,457,013. Preferred metal oxides are antimony doped tin oxide, aluminum doped zinc oxide, niobium doped titanium oxide, and metal antimonates. These patents do not teach any specific requirements for the binder polymer and, as a result, there is a need for a high volume % of the conductive fine particles in the conductive coatings in order to achieve effective antistatic performance. This results in reduced transparency due to scattering losses and in brittle films subject to cracking and poor adherence to the support material.

JP A4055492 describes antistatic layers comprising conductive non-oxide particles including TiN, NbB<sub>2</sub>, TiC, and MoB dispersed in a binder such as a water soluble polymer or solvent soluble resin.

U.S. Pat. No. 5,066,422 describes vinyl surface covering materials comprising a fused sheet of a dry blend, wherein the dry blend contains a polyvinyl chloride porous resin, a

plasticizer, and conductive particles. Reportedly, the conductive particles reside in the pores and surface of the polyvinyl chloride resin which thereby provides surface resistivities of the fused sheet of  $10^9 \Omega$  per square at low weight % of the conductive particles.

Fibrous conductive powders comprising antimony doped tin oxide coated onto nonconductive potassium titanate whiskers have been used to prepare conductive layers for photographic and electrographic applications. Such materials have been disclosed in U.S. Pat. No. 4,845,369, U.S. Pat. No. 5,116,666, JP A63098656, and JP A63060452. Layers containing these conductive whiskers dispersed in a binder reportedly provide improved conductivity at lower volume % than the aforementioned conductive fine particles as a result of their higher aspect (length to diameter) ratio. However, the benefits obtained as a result of the reduced volume % requirements are offset by the fact that these materials are large in size (10 to 20  $\mu\text{m}$  long and 0.2-0.5  $\mu\text{m}$  diameter). The large size results in increased light scattering and hazy coatings.

Transparent, binderless, electrically semiconductive metal oxide thin films formed by oxidation of thin metal films which have been vapor deposited onto film base are described in U.S. Pat. No. 4,078,935. The resistivity of such conductive thin films have been reported to be  $10^5 \Omega$  per square. However, these metal oxide thin films are unsuitable for photographic film applications since the overall process used to prepare them is complex and expensive and adhesion of these thin films to the film base and overlying layers is poor.

U.S. Pat. No. 4,203,769 describes an antistatic layer incorporating "amorphous" vanadium pentoxide. This vanadium pentoxide antistat is highly entangled, high aspect ratio ribbons 50-100 Angstroms wide, about 10 Angstroms thick, and 0.1-1  $\mu\text{m}$  long. As a result of this ribbon structure surface resistivities of  $10^6$ - $10^{11} \Omega$  per square can be obtained for coatings containing very low volume fractions of vanadium pentoxide. This results in very low optical absorption and scattering losses, thus the coatings are highly transparent and colorless. However, vanadium pentoxide is soluble at the high pH typical of film developer solutions and must be overcoated with a nonpermeable barrier layer to maintain antistatic performance after film processing.

It can be seen that a variety of methods have been reported in an attempt to obtain non-brittle, adherent, highly transparent, colorless conductive coatings with humidity independent, film process surviving antistatic performance. The aforementioned prior art references relate to some aspects of the present invention, but, they are deficient with regard to simultaneously satisfying all of the above mentioned requirements.

U.S. Pat. No. 5,340,676 describes conductive layers comprising electrically-conductive fine particles, hydrophilic colloid, and water-insoluble polymer particles. Representative polymer particles described include polymers and interpolymers of styrene, styrene derivatives, alkyl acrylates or alkyl methacrylates and their derivatives, olefins, vinylidene chloride, acrylonitrile, acrylamide and methacrylamide derivatives, vinyl esters, vinyl ethers, or condensation polymers such as polyurethanes and polyesters. The use of a mixed binder comprising the polymer particles mentioned above in combination with a hydrophilic colloid such as gelatin provides a conductive coating that requires lower volume % conductive fine particles compared with a layer obtained from a coating composition comprising the conductive fine particles and water soluble hydrophilic colloid

alone. Copending commonly-assigned U.S. Provisional Patent Application Ser. No. 60/000236, filed Jun. 15, 1995, describes a further improvement to the '676 patent in that the water-insoluble polymer particles are gelatin-grafted polymer particles. The use of gelatin-grafted polymer particles improves the stability of the coating formulation. U.S. Pat. No. 5,466,567 describes conductive layers comprising electrically-conductive fine particles, hydrophilic colloid, and water-insoluble, precrosslinked gelatin particles.

Electrically-conductive layers prepared from coating compositions described in the '676 patent, application Ser. No. 60/000236 and the '567 patent are especially useful when the conductive layer is to be overcoated with a layer containing a hydrophilic colloid.

It is toward the objective of providing a new and improved electrically-conductive layer that is capable of utilizing low volume percentages of the electrically-conductive fine particles that the present invention is directed. Use of such low volume percentages provides improved layer transparency since most of the known electrically-conductive fine particles have a high refractive index or are highly colored. In addition, minimizing the amount of electrically-conductive fine particles incorporated into a dried coating, especially for conductive metal oxide particles, can provide improved physical properties (e.g., freedom from brittleness), reduced cost for the coated layer, and reduced finishing tool wear.

## SUMMARY OF THE INVENTION

In accordance with this invention, an imaging element for use in an image-forming process comprises a support, an image-forming layer, and an electrically-conductive layer. The electrically-conductive layer consists essentially of electrically-conductive fine particles and as a binder, water-insoluble polymer particles. The water-insoluble polymer particles that serve as the binder in the electrically-conductive layer comprise polymers having a sulfonic acid group.

The combination of electrically-conductive fine particles and water-insoluble polymer particles that have a sulfonic acid group provides conductive coatings which can employ low volume percentages of conductive particles and still provide the desired high degree of conductivity.

## DETAILED DESCRIPTION OF THE INVENTION

The imaging elements of this invention can be of many different types depending on the particular use for which they are intended. Such elements include, for example, photographic, electrostatographic, photothermographic, migration, electrothermographic, dielectric recording and thermal-dye-transfer imaging elements.

Details with respect to the composition and function of a wide variety of different imaging elements are provided in U.S. Pat. No. 5,340,676 and references described therein. The present invention can be effectively employed in conjunction with any of the imaging elements described in the '676 patent.

Photographic elements represent an important class of imaging elements within the scope of the present invention. In such elements, the electrically-conductive layer may be applied as a subbing layer, an intermediate layer, or as the outermost layer on the sensitized emulsion side of the support, on the side of the support opposite the emulsion, or on both sides of the support. The support may comprise any commonly used photographic support material such as

polyester, cellulose acetate, or resin-coated paper. The electrically-conductive layer is applied from a coating formulation consisting essentially of electrically-conductive fine particles and water-insoluble polymer particles. The conductive fine particle can be, for example, a doped-metal oxide, a metal oxide containing oxygen deficiencies, a metal antimonate, or a conductive nitride, carbide, or boride. Representative examples of conductive fine particles include conductive  $TiO_2$ ,  $SnO_2$ ,  $Al_2O_3$ ,  $ZrO_3$ ,  $In_2O_3$ ,  $MgO$ ,  $ZnSb_2O_6$ ,  $InSbO_4$ ,  $TiB_2$ ,  $ZrB_2$ ,  $NbB_2$ ,  $TaB_2$ ,  $CrB_2$ ,  $MoB$ ,  $WB$ ,  $LaB_6$ ,  $ZrN$ ,  $TiN$ ,  $TiC$ , and  $WC$ . The conductive fine particle may also be an electrically conductive polymer particle comprising inherently conductive polymers such as polyacetylenes, polyanilines, polythiophenes and polypyrrroles. The conductive fine particle preferably has an average particle size less than about  $0.3\text{ }\mu\text{m}$  and a powder resistivity of  $10^5\text{ }\Omega\text{ cm}$  or less.

The water-insoluble polymer particles in accordance with the present invention preferably have an average size of from 10 nm to 1000 nm, and more preferably from 20 to 500 nm. The polymer particle can be a homopolymer or copolymer particle prepared by emulsion polymerization of ethylenically unsaturated monomers. The sulfonic acid groups are incorporated into at least part of the polymers by using an effective amount of ethylenically unsaturated monomers having a sulfonic acid group. Representative ethylenically unsaturated monomers include, for example, styrene and its derivatives, alkyl acrylates or alkyl methacrylates and their derivatives, olefins, vinylidene chloride, acrylonitrile, acrylamide and methacrylamide derivatives, vinyl esters, and vinyl ethers. In addition, crosslinking monomers such as 1,4-butyleneglycol methacrylate, trimethylolpropane triacrylate, allyl methacrylate, diallyl phthalate, divinyl benzene, and the like may be used in order to give a crosslinked polymer particle. Representative ethylenically unsaturated monomers having a sulfonic acid group include, for example, styrenesulfonic acid, vinyl sulfonic acid, 2-methacryloyloxyethyl-1-sulfonic acid, 2-acrylamido-2-methylpropane sulfonic acid, 3-methacryloyloxypropane-1-methyl-1-sulfonic acid, 3-methacryloyloxypropane-1-sulfonic acid, and the like. Chain transfer agents including mercaptans, polymercaptans, and halogen compounds can be used in the polymerization mixture to moderate the polymer molecular weight. The weight average molecular weight of the polymers may vary from 5,000 to 30,000,000 and preferably from 10,000 to 10,000,000. The polymer particle useful for the present invention can also be prepared by post emulsification of preformed polymers, in which the preformed polymers may be first dissolved together with an effective amount of preformed polymers having a sulfonic acid group in an organic solvent and then the polymer solution is emulsified in an aqueous media in the presence of an appropriate emulsifier. The polymer particle may also be a water dispersible condensation polymer such as a polyurethane, polyester, or polyamide. The polymer particle useful for the present invention preferably has an acid number (the number of milligrams of KOH required to neutralize 1 g of solid polymer particles) in the range of from 1.5 to 70, more preferably from 1.5 to 60, most preferably from 6 to 30. The sulfonic acid groups attached to the polymer particle are preferably in a neutralized form, i.e. salt, for example, alkali metal salts, alkali earth metal salts, ammonium salts, and substituted or unsubstituted alkyl amine salts having 1 to 10 carbon atoms.

Sulfonic-acid-group-containing binders for electronically-conductive agents have been described in U.S. Pat. Nos. 5,203,884, 5,360,706, 5,372,985, 5,424,269,

5,427,835, 5,439,785 and 5,468,498. However, in these patents the conductive agent is fibrous  $V_2O_5$  rather than a conductive fine particle. Since  $V_2O_5$  is fibrous in nature, it can be used at extremely low volume percentages regardless of the nature of the polymer binder. In the aforementioned patents, a sulfopolymer is used to improve the stability of the  $V_2O_5$ -containing coating formulation. In the present invention for electrically-conductive layers containing conductive fine particles it has been unexpectedly discovered that water-insoluble polymer particles comprising a sulfonic acid group allow reduction in the volume percentage of the conductive fine particles.

The latex copolymer particle prepared by an emulsion polymerization process can have various microstructures or morphologies that include perfectly homogeneous copolymers prepared in a well controlled semicontinuous process, a core/shell morphology using a multistage polymerization process, or more complex structures with distribution gradients or even matrix inclusion structures (Daniel, J. C., 15 Makromol. Chem. Suppl 10/11. 359, 1985). For core/shell polymer particles, the sulfonic acid group is preferably incorporated into the particle shell.

The polymer particles useful for the present invention 25 may include reactive functional groups capable of forming covalent bonds by intermolecular crosslinking or by crosslinking reaction with a crosslinking agent. Suitable reactive functional groups include: hydroxyl, carboxyl, 30 amino, amide, allyl, carbodiimide, epoxide, aziridine, vinyl sulfone, sulfonic acid, active methylene, and the like.

Up to 30 weight % of the total polymer particle binder 35 weight may comprise polymer particles other than those that contain ethylenically unsaturated monomers having a sulfonic acid group without significantly affecting the benefits of the present invention.

The coating compositions of the invention may also 40 contain suitable crosslinking agents including aldehydes, epoxy compounds, polyfunctional aziridines, vinyl sulfones, methoxyalkyl melamines, triazines, polyisocyanates, dioxane derivatives such as dihydroxydioxane, carbodiimides, and the like. The crosslinking agents may react with functional groups present on the polymer particle binder in the coating composition.

Matte particles well known in the art may also be used in 45 the coating compositions of the invention, such matting agents have been described in Research Disclosure No. 308, published December 1989, pages 1008 to 1009. When polymer matte particles are employed, the polymer may contain reactive functional groups capable of forming covalent bonds with the binder polymer by intermolecular crosslinking or by reaction with a crosslinking agent in order 50 to promote improved adhesion of the matte particles to the coated layers. Suitable reactive functional groups include: hydroxyl, carboxyl, carbodiimide, epoxide, aziridine, vinyl sulfone, sulfonic acid, active methylene, amino, amide, allyl, and the like.

The coating compositions of the present invention may 55 also include lubricants or combinations of lubricants to reduce sliding friction of the image elements in accordance 60 with the invention. Typical lubricants include (1) silicone based materials disclosed, for example, in U.S. Pat. Nos. 3,489,567, 3,080,317, 3,042,522, 4,004,927, and 4,047,958, and in British Patent Nos. 955,061 and 1,143,118; (2) higher fatty acids and derivatives, higher alcohols and derivatives, metal salts of higher fatty acids, higher fatty acid esters, higher fatty acid amides, polyhydric alcohol esters of higher fatty acids, etc disclosed in U.S. Pat. Nos. 2,454,043,

2,732,305, 2,976,148, 3,206,311, 3,933,516, 2,588,765, 3,121,060, 3,502,473, 3,042,222, and 4,427,964, in British Patent Nos. 1,263,722, 1,198,387, 1,430,997, 1,466,304, 1,320,757, 1,320,565, and 1,320,756, and in German Patent Nos. 1,284,295 and 1,284,294; (3) liquid paraffin and paraffin or wax like materials such as carnauba wax, natural and synthetic waxes, petroleum waxes, mineral waxes and the like; (4) perfluoro- or fluoro- or fluorochloro-containing materials, which include poly(tetrafluoroethylene), poly(trifluorochloro-ethylene), poly(vinylidene fluoride, poly(trifluoro-chloroethylene-co-vinyl chloride), poly(meth)acrylates or poly(meth)acrylamides containing perfluoroalkyl side groups, and the like. Lubricants useful in the present invention are described in further detail in Research Disclosure No.308, published December 1989, page 1006.

The coating compositions of the invention may be applied to the support material by any coating method well known in the art, for example, hopper coating, gravure coating, roller coating, air knife coating, spray coating, etc. The coatings may be dried using a wide range of drying conditions. Preferably, the coatings are dried by impingement with air that has a temperature of at least 100° C. These high drying temperatures are desirable for high speed coating and drying and provide improved adhesion to the support materials employed in the photographic industry.

The conductive layer preferably comprises 50 volume % or less of the conductive fine particles, more preferably 35 volume % or less of the conductive fine particles. The amount of the conductive particle contained in the coating is defined in terms of volume % rather than weight % since the densities of the conductive particles and polymer binders may differ widely. The binder for the conductive particles comprises the water-insoluble polymer particles with the specific characteristics described above. The layer can additionally contain wetting aids, biocides, dispersing aids, antifoam agents, soluble or solid particle dyes, magnetic particles, and coalescing aids. The conductive layer is applied from an aqueous coating formulation to give dried coating weights preferably of about 100 to 1500 mg/m<sup>2</sup>.

In a particularly preferred embodiment, the imaging elements of this invention are photographic elements, such as photographic films, photographic papers or photographic glass plates, in which the image-forming layer is a radiation-sensitive silver halide emulsion layer. Such emulsion layers typically comprise a film-forming hydrophilic colloid. The most commonly used of these is gelatin and gelatin is a particularly preferred material for use in this invention. Useful gelatins include alkali-treated gelatin (cattle bone or hide gelatin), acid-treated gelatin (pigskin gelatin) and gelatin derivatives such as acetylated gelatin, phthalated gelatin and the like. Other hydrophilic colloids that can be utilized alone or in combination with gelatin include dextran, gum arabic, zein, casein, pectin, collagen derivatives, collodion, agar-agar, arrowroot, albumin, and the like. Still other useful hydrophilic colloids are water-soluble polyvinyl compounds such as polyvinyl alcohol, polyacrylamide, poly(vinylpyrrolidone), and the like.

The photographic elements of the present invention can be simple black-and-white or monochrome elements comprising a support bearing a layer of light-sensitive silver halide emulsion or they can be multilayer and/or multicolor elements.

Color photographic elements of this invention typically contain dye image-forming units sensitive to each of the three primary regions of the spectrum. Each unit can be

comprised of a single silver halide emulsion layer or of multiple emulsion layers sensitive to a given region of the spectrum. The layers of the element, including the layers of the image-forming units, can be arranged in various orders as is well known in the art.

A preferred photographic element according to this invention comprises a support bearing at least one blue-sensitive silver halide emulsion layer having associated therewith a yellow image dye-providing material, at least one green-sensitive silver halide emulsion layer having associated therewith a magenta image dye-providing material and at least one red-sensitive silver halide emulsion layer having associated therewith a cyan image dye-providing material.

In addition to emulsion layers, the elements of the present invention can contain auxiliary layers conventional in photographic elements, such as overcoat layers, spacer layers, filter layers, interlayers, antihalation layers, pH lowering layers (sometimes referred to as acid layers and neutralizing layers), timing layers, opaque reflecting layers, opaque light-absorbing layers and the like. The support can be any suitable support used with photographic elements. Typical supports include polymeric films, paper (including polymer-coated paper), glass and the like. Details regarding supports and other layers of the photographic elements of this invention are contained in *Research Disclosure*, Item 36544, September, 1994.

The light-sensitive silver halide emulsions employed in the photographic elements of this invention can include coarse, regular or fine grain silver halide crystals or mixtures thereof and can be comprised of such silver halides as silver chloride, silver bromide, silver bromoiodide, silver chlorobromide, silver chloroiodide, silver chlorobromoiodide, and mixtures thereof. The emulsions can be, for example, tabular grain light-sensitive silver halide emulsions. The emulsions can be negative-working or direct positive emulsions. They can form latent images predominantly on the surface of the silver halide grains or in the interior of the silver halide grains. They can be chemically and spectrally sensitized in accordance with usual practices. The emulsions typically will be gelatin emulsions although other hydrophilic colloids can be used in accordance with usual practice. Details regarding the silver halide emulsions are contained in *Research Disclosure*, Item 36544, September, 1994, and the references listed therein.

The photographic silver halide emulsions utilized in this invention can contain other addenda conventional in the photographic art. Useful addenda are described, for example, in *Research Disclosure*, Item 36544, September, 1994. Useful addenda include spectral sensitizing dyes, desensitizers, antifoggants, masking couplers, DIR couplers, DIR compounds, antistain agents, image dye stabilizers, absorbing materials such as filter dyes and UV absorbers, light-scattering materials, coating aids, plasticizers and lubricants, and the like.

Depending upon the dye-image-providing material employed in the photographic element, it can be incorporated in the silver halide emulsion layer or in a separate layer associated with the emulsion layer. The dye-image-providing material can be any of a number known in the art, such as dye-forming couplers, bleachable dyes, dye developers and redox dye-releasers, and the particular one employed will depend on the nature of the element, and the type of image desired.

Dye-image-providing materials employed with conventional color materials designed for processing with separate solutions are preferably dye-forming couplers; i.e., com-

pounds which couple with oxidized developing agent to form a dye. Preferred couplers which form cyan dye images are phenols and naphthols. Preferred couplers which form magenta dye images are pyrazolones and pyrazolotriazoles. Preferred couplers which form yellow dye images are benzoylacetanilides and pivalylacetanilides.

The invention is further illustrated by the following examples of its practice.

#### EXAMPLE 1

Two ethyl methacrylate-containing polymers were prepared by a conventional emulsion polymerization process. The composition and particle size for the polymer particles are shown in Table 1. Particle P-2 has an acid number equal to 21.

TABLE 1

| Par- | Polymer Composition                                                                                           | Particle Size (nm) |
|------|---------------------------------------------------------------------------------------------------------------|--------------------|
| P-1  | ethyl methacrylate/methacrylic acid 95/5                                                                      | 75                 |
| P-2  | ethyl methacrylate/sodium acrylamido-2-methylpropane sulfonate/2-acetoacetoxy ethyl methacrylate 88.9/7.6/3.5 | 78                 |

Conductive coatings comprising conductive fine particles and polymer binder were coated onto 4 mil thick polyethylene terephthalate film support that had been subbed with a terpolymer latex of acrylonitrile, vinylidene chloride, and acrylic acid. The aqueous coating formulations comprising about 4 weight % total solids were dried at 100° C. to give dried coating weights of 1000 mg/m<sup>2</sup>. The coatings contained 10 or 20 volume % of conductive tin oxide particles (doped with 6% antimony) with an average primary particle size of about 15 nm.

The surface resistivity of the coatings was measured at 20% relative humidity using a 2-point probe. The coating compositions and resistivities for the coatings are tabulated in Table 2. As can be seen from the results, coating compositions of the invention that contain a water-insoluble polymer particle binder having a sulfonic acid group provide resistivity values that are as much as one order of magnitude superior to the comparative coating compositions.

Dry adhesion of the conductive layers to the support was determined by scribing small hatch marks in the coating with a razor blade, placing a piece of high tack tape over the scribed area and then quickly pulling the tape from the surface. The amount of the scribed area removed is a measure of the dry adhesion. Wet adhesion for the coatings was tested by placing the test samples in deionized water at 35° C. for 1 minute. While still wet, a one millimeter wide line was scribed in the coating and a finger was rubbed vigorously across the scribe line. The percent of the rubbed area that was removed was used as a measure of wet adhesion. The wet and dry adhesion for the coatings of the invention were found to be excellent.

TABLE 2

|             | Coating No. | Binder | Volume % SnO <sub>2</sub> | Surface Resistivity (Ω per sq) |
|-------------|-------------|--------|---------------------------|--------------------------------|
| Comparative | 1           | P-1    | 10                        | 4.0 × 10 <sup>10</sup>         |
| Invention   | 2           | P-2    | 10                        | 4.0 × 10 <sup>9</sup>          |

TABLE 2-continued

|             | Coating No. | Binder | Volume % SnO <sub>2</sub> | Surface Resistivity (Ω per sq) |
|-------------|-------------|--------|---------------------------|--------------------------------|
| Comparative | 3           | P-1    | 20                        | 1.0 × 10 <sup>9</sup>          |
| Invention   | 4           | P-2    | 20                        | 4.0 × 10 <sup>8</sup>          |

10

#### EXAMPLE 2

Five butyl methacrylate-containing polymers were prepared by a conventional emulsion polymerization process. The compositions for these polymer particles are shown in Table 3. The particle size for these particles was 60 to 80 nm. Particles P-5, P-6, and P-7 have an acid number equal to 14.7, 15.5, and 13.8, respectively.

TABLE 3

| Particle | Polymer Composition                                                 |
|----------|---------------------------------------------------------------------|
| P-3      | butyl methacrylate                                                  |
| P-4      | butyl methacrylate/methacrylic acid 95/5                            |
| P-5      | butyl methacrylate/2-sulfoethyl methacrylate 95/5                   |
| P-6      | butyl methacrylate/sodium styrene sulfonate 95/5                    |
| P-7      | butyl methacrylate/sodium acrylamido-2-methylpropane sulfonate 95/5 |

20

Conductive layers were prepared from coating compositions containing conductive tin oxide particles and the butyl methacrylate polymer particles described in Table 3. The coatings were applied onto the aforementioned polyester support and dried at 100° C. to give conductive layers with a dried coating weight of 1000 mg/m<sup>2</sup>. The surface resistivity for the coatings was measured at 20% relative humidity and the results reported in Table 4.

As seen by the results given in Table 4, coatings of the invention containing either particles P-5, P-6, or P-7 that contain sulfonic acid groups provide superior resistivity results compared with comparative coatings containing similar butyl methacrylate particles without sulfonic acid groups. Also, it can be seen by comparing the results for coatings 8, 12, 16, 20, and 24 that the benefits of utilizing polymer particles that contain sulfonic acid groups are insignificant at high conductive particle concentrations (i.e., >50 volume %). While it is known that sulfonic acid-containing polymers are useful as antistatic materials (at high humidities) as a result of their ionic conductivity it was not obvious prior to the present invention that sulfonic acid-containing polymer particles would improve the low humidity conductivity of coating compositions containing electronically conductive fine particles. Although the exact mechanism is not fully understood we believe that the presence of the sulfonic acid group on the polymer particles enhances the formation of an electrically conductive network of the conductive fine particles. At low humidity (e.g., 20 % relative humidity) and the low concentrations of the sulfonic acid groups contained in the polymer particles it is unlikely that the improvement in the conductivity of the coatings of the invention is a result of the ionic conductivity of the polymer particles.

25

30

35

40

45

50

55

60

65

TABLE 4

| Coating No.    | Binder | Volume % SnO <sub>2</sub> | Surface Resistivity (Ω per sq) |
|----------------|--------|---------------------------|--------------------------------|
| Comparative 5  | P-3    | 5                         | 3.0 × 10 <sup>13</sup>         |
| Comparative 6  | P-3    | 9                         | 1.3 × 10 <sup>11</sup>         |
| Comparative 7  | P-3    | 29                        | 5.0 × 10 <sup>8</sup>          |
| Comparative 8  | P-3    | 60                        | 1.2 × 10 <sup>8</sup>          |
| Comparative 9  | P-4    | 5                         | >1.0 × 10 <sup>14</sup>        |
| Comparative 10 | P-4    | 9                         | 2.5 × 10 <sup>11</sup>         |
| Comparative 11 | P-4    | 29                        | 6.3 × 10 <sup>8</sup>          |
| Comparative 12 | P-4    | 60                        | 1.6 × 10 <sup>8</sup>          |
| Invention 13   | P-5    | 5                         | 1.0 × 10 <sup>13</sup>         |
| Invention 14   | P-5    | 9                         | 3.1 × 10 <sup>10</sup>         |
| Invention 15   | P-5    | 29                        | 1.6 × 10 <sup>8</sup>          |
| Comparative 16 | P-5    | 60                        | 1.0 × 10 <sup>8</sup>          |
| Invention 17   | P-6    | 5                         | 7.9 × 10 <sup>11</sup>         |
| Invention 18   | P-6    | 9                         | 4.0 × 10 <sup>10</sup>         |
| Invention 19   | P-6    | 29                        | 2.0 × 10 <sup>8</sup>          |
| Comparative 20 | P-6    | 60                        | 1.0 × 10 <sup>8</sup>          |
| Invention 21   | P-7    | 5                         | 4.0 × 10 <sup>11</sup>         |
| Invention 22   | P-7    | 9                         | 2.0 × 10 <sup>10</sup>         |
| Invention 23   | P-7    | 29                        | 2.0 × 10 <sup>8</sup>          |
| Comparative 24 | P-7    | 60                        | 1.0 × 10 <sup>8</sup>          |

The invention has been described in detail with particular reference to certain preferred embodiments thereof, but it will be understood that variations and modifications can be effected within the spirit and scope of the invention.

We claim:

1. An imaging element for use in an image-forming process; said imaging element comprising a support, an image-forming layer, and an electrically-conductive layer; said electrically-conductive layer consisting essentially of electrically-conductive fine particles and as a binder water-insoluble polymer particles wherein at least 70% of the water-insoluble polymer particles must contain ethylenically unsaturated monomers having a sulfonic acid group.

2. An imaging element as claimed in claim 1, wherein said electrically-conductive fine particles are composed of a doped-metal oxide, a metal oxide containing oxygen deficiencies, a metal antimonate, or a conductive nitride, carbide or boride.

3. An imaging element as claimed in claim 1, wherein said electrically-conductive fine particles are antimony-doped tin oxide particles.

4. An imaging element as claimed in claim 1, wherein said electrically-conductive fine particles have an average particle size of less than about 0.3 mm and a powder resistivity of 10<sup>5</sup> Ω·cm or less.

5. An imaging element as claimed in claim 1, wherein said water-insoluble polymer particles have an average diameter of from about 10 nm to about 1000 nm.

6. An imaging element as claimed in claim 1, wherein said water-insoluble polymer particles have an average diameter of from 20 nm to 500 nm.

7. An imaging element as claimed in claim 1, wherein said water-insoluble polymer particles have an acid number of from 1.5 to 70.

8. An imaging element as claimed in claim 1, wherein said water-insoluble polymer particles have an acid number of from 6 to 30.

9. An imaging element as claimed in claim 1, wherein said sulfonic acid groups are in neutralized form.

10. An imaging element as claimed in claim 1, wherein said water-insoluble polymer particles are selected from the group consisting of polymers of styrene, derivatives of styrene, alkyl acrylates, derivatives of alkyl acrylates, alkyl methacrylates, derivatives of alkyl methacrylates, itaconic

acid, derivatives of itaconic acid, olefins, vinylidene chloride, acrylonitrile, acrylamide, derivatives of acrylamide, methacrylamide, derivatives of methacrylamide, vinyl esters, vinyl ethers and urethanes.

5 11. An imaging element as claimed in claim 1, wherein said water-insoluble polymer particles are polymers of an ethylenically unsaturated monomer selected from the group consisting of styrenesulfonic acid, vinyl sulfonic acid, 2-methacryloyloxyethyl-1-sulfonic acid, 2-acrylamido-2-methylpropane sulfonic acid, 3-methacryloyloxypropane-1-methyl-1-sulfonic acid and 3-methacryloyloxypropane-1-sulfonic acid.

10 12. An imaging element as claimed in claim 1, wherein said water-insoluble polymer particles are particles of an interpolymer of ethyl methacrylate, sodium acrylamido-2-propane sulfonate and 2-acetoacetoxy ethyl methacrylate.

15 13. An imaging element as claimed in claim 1, wherein said water-insoluble polymer particles are particles of a copolymer of butyl methacrylate and 2-sulfoethyl methacrylate.

20 14. An imaging element as claimed in claim 1, wherein said water-insoluble polymer particles are particles of a copolymer of butyl methacrylate and sodium styrene sulfonate.

25 15. An imaging element as claimed in claim 1, wherein said water-insoluble polymer particles are particles of a copolymer of butyl methacrylate and sodium acrylamido-2-propane sulfonate.

16. An imaging element as claimed in claim 1, wherein said electrically-conductive layer comprises 50 volume % or less of said electrically-conductive fine particles.

30 17. An imaging element as claimed in claim 1, wherein said electrically-conductive layer comprises 35 volume % or less of said electrically-conductive fine particles.

35 18. An imaging element as claimed in claim 1, wherein the dry coating weight of said electrically-conductive layer is in the range of from about 100 to about 1500 mg/m<sup>2</sup>.

19. An imaging element as claimed in claim 1, wherein said support is a polyethylene terephthalate film.

20. A photographic film comprising:

(1) a support;  
 (2) an electrically-conductive layer which serves as an antistatic layer overlying said support; and  
 (3) a silver halide emulsion layer overlying said electrically-conductive layer; said electrically-conductive layer consisting essentially of electrically-conductive fine particles and as a binder water-insoluble polymer particles wherein at least 70 percent of the water-insoluble polymer particles must contain ethylenically unsaturated monomers having a sulfonic acid group.

21. A photographic film comprising a cellulose ester or polyester support, an image-forming layer comprising a silver halide emulsion, and an electrically-conductive layer which serves as an antistatic layer; said electrically-conductive layer consisting essentially of electrically-conductive fine particles having an average particle size of less than about 0.3 mm and a powder resistivity of 10<sup>5</sup> Ω·cm or less and as a binder water-insoluble polymer particles wherein at least 70 percent of the water-insoluble polymer particles must contain ethylenically unsaturated monomers having a sulfonic acid group having an average diameter of from 20 nm to 500 nm, wherein said electrically-conductive layer comprises 50 volume % or less of said electrically-conductive fine particles.